

1

2,749,239

## ALUMINUM BASE ALLOY

Walter E. Sicha, Shaker Heights, and Harold Y. Hunsicker and Robert C. Lemon, Cleveland, Ohio, assignors to Aluminum Company of America, Pittsburgh, Pa., a corporation of Pennsylvania

No Drawing. Application March 14, 1955,  
Serial No. 494,264

6 Claims. (Cl. 75—142)

This invention relates to the composition of improved aluminum base alloys which in cast form are especially suited for service at higher temperatures than have been considered heretofore to be feasible for aluminum base alloys.

Aluminum base alloys have been employed in the manufacture of many articles which have been exposed to a wide variety of service conditions. For the most part, this has involved service at temperatures below 400° F., and generally at room temperature. With the introduction and progress of jet and diesel engines as well as other devices which operate at high temperatures, it was found that the previous alloys did not have the requisite properties for satisfactory performance. Extensive investigations have been made to find new compositions which would better meet the new requirements. Special attention has been given to alloys which can be readily cast and do not require the presence of high cost alloying elements.

It is accordingly an object of this invention to provide an aluminum base alloy casting which possesses superior strength and hardness at temperatures on the order of 600 to 700° F. Another object is to provide an aluminum base alloy casting which does not require thermal treatment to develop its maximum strength at elevated temperatures. Still another object is to provide an aluminum base alloy casting which possesses superior fatigue properties at elevated temperatures. A further object is to provide an alloy casting which undergoes substantially no permanent change in dimensions as a result of exposure to elevated temperatures.

These and other objects and advantages are realized in castings of an aluminum base alloy which contains copper, magnesium, manganese and nickel as the primary added alloying components. We have discovered that unique and unusual properties are obtained in an alloy which, in addition to aluminum and impurities, contains from 6 to 18% copper, 4 to 8% magnesium, 0.1 to 2% manganese and 0.1 to 2% nickel, the proportion between copper and magnesium being such that the amount of copper equals or exceeds the magnesium content. Alloys within the foregoing range can be melted and cast in accordance with usual practices, require no solution heat treatment prior to being placed in service to develop maximum properties and possess a higher strength and hardness at temperatures on the order of 600 to 700° F. than exhibited by the commercial aluminum base alloys previously used for such articles as pistons, cylinder heads and the like. Castings of our alloy have a tensile strength at 600° F. of not less than 15,000 p. s. i. in the as-cast condition. In addition, the cast alloy has a fatigue strength at 600° F., on the order of 8,000 p. s. i. at 10<sup>7</sup> cycles, which is much higher than that of prior well known aluminum base alloys.

The copper content of the alloys, 6 to 18%, which is higher than that found in most alloys of the aluminum-copper type, should not be less than the magnesium content. For best results, the copper should be within

2

the range of 7 to 11% and should exceed the amount of magnesium present. It is also preferred that the total amount of magnesium, nickel and manganese should be less than the copper content.

Although the quantity of magnesium used in the alloy should never exceed the amount of copper present, magnesium is still an important component of the alloy. In combination with copper it provides the basic characteristics of the alloy which adapt it to service at elevated temperatures. Hitherto, magnesium has been employed in relatively small amounts in aluminum-copper type alloys, especially those which are subjected to solution heat treatment and precipitation hardening to develop maximum strength and hardness. In the present case, from 4 to 8% should be employed, but optimum results are obtained if the range is confined to between 5 and 7%. Particularly advantageous properties are developed where the proportion of magnesium to copper is such that the magnesium content is at least one-half the copper content and the copper does not exceed 16%. When the preferred proportions of the two elements are employed the tensile strength at 600° F. is not less than 17,000 p. s. i.

The manganese and nickel components are necessary to produce the required properties of the alloy at high temperatures, although the quantities used are relatively small. As mentioned above, the amount of each element should be between 0.1 and 2% but in our preferred practice from 0.4 to 1% should be employed. Moreover, for optimum results the two elements should be used in substantially equal amounts.

As is well recognized in the aluminum base alloy art, it is often desirable to add minor quantities of certain elements to improve certain characteristics such as grain size or resistance to oxidation. For example, the presence of 0.001 to 0.1% boron or 0.01 to 0.2% titanium, or both, will serve to reduce the grain size while the addition of 0.0001 to 0.1% beryllium imparts resistance to oxidation. Another group of elements, which may be called supplementary hardening agents, which we have found can be used to advantage consists of chromium, cobalt, molybdenum, tungsten, zirconium and vanadium. These elements may be used individually in amounts of 0.1 to 0.6%, but where two or more are employed, the total quantity should not exceed 1.0%.

The aluminum employed in making the alloy may be of the purity normally used in making castings. Generally, the iron impurity contents of the alloy should not exceed 1% and the silicon impurity should not be over 0.75%. It is to be understood that traces of other elements may also be present but they can be disregarded for present purposes.

Our alloy may be melted and cast in accordance with conventional procedures and hence it is well adapted to use with existing equipment. Furthermore it can be readily cast in sand or permanent molds.

The alloys herein described do not require any solution heat treatment to develop the desired properties at elevated temperatures. This is an important advantage both from the standpoint of cost and stability at high temperatures. In respect to the latter feature, it may be mentioned that the beneficial effects of solution heat treatment of other alloys can be dissipated upon long exposure to elevated temperatures but this effect would not be encountered with our alloy since it does not require such preliminary treatment. For some purposes it has been found to be desirable to subject the cast alloy to a stabilizing thermal treatment to relieve any internal stresses. This involves heating the castings for a period of 2 to 5 hours at a temperature between 550 and 700° F.

One of the important features of the castings made from our alloy is that they do not exhibit any significant

permanent dimensional changes upon long exposure to elevated temperatures. The castings are therefore free from the objectionable "growth" which has characterized many previous casting alloys when used at temperatures on the order of 400° F. and higher.

The advantages and benefits of our invention can be better appreciated by referring to the elevated temperature properties of castings of some representative alloys in comparison with the properties of the same type of casting made from Y alloy, a composition long regarded as being particularly adapted for elevated temperature service. Melts of the various alloys were prepared in accordance with conventional practice and poured in sand tensile test bar molds, and the castings cooled to room temperature. A portion of the bars were heated to 600° F., held at that temperature for 48 hours and tested while at temperature. The alloy compositions and average tensile properties of the cast bars are given in Table I below.

TABLE I

Tensile properties of various alloy castings at 600° F.

| Composition, Percent |     |     |             | Tensile Strength, p. s. i. | Yield Strength, p. s. i. | Elongation, percent in 2 in. |
|----------------------|-----|-----|-------------|----------------------------|--------------------------|------------------------------|
| Cu                   | Mg  | Mn  | Ni          |                            |                          |                              |
| 10                   | 4   | 0.5 | 0.5         | 19,500                     | 12,000                   | 5                            |
| 10                   | 6   | 0.5 | 0.5         | 20,500                     | 13,000                   | 25                           |
| 10                   | 8   | 0.5 | 0.5         | 18,000                     | 13,000                   | 20                           |
| 6                    | 6   | 0.5 | 0.5         | 18,000                     | 12,500                   | 30                           |
| 8                    | 6   | 0.5 | 0.5         | 19,500                     | 14,500                   | 25                           |
| 14                   | 6   | 0.5 | 0.5         | 23,500                     | 14,500                   | 1.0                          |
| 8                    | 6   | 0.5 | 1.0         | 18,500                     | 11,700                   | 14                           |
| 8                    | 6   | 1.0 | 1.5         | 19,100                     | 11,200                   | 5                            |
| 8                    | 6   | 1.5 | 1.5         | 20,500                     | 11,000                   | 5                            |
| 8                    | 6   | 1.5 | 2.0         | 19,500                     | 11,300                   | 4                            |
| 4                    | 1.5 | --  | 2 (Y alloy) | 12,500                     | 8,000                    | 5                            |

It is to be noted that the tensile strength increases with the copper content and that higher tensile strength values were obtained in those alloys in which the copper exceeded the magnesium content. It is also apparent that the elongation diminishes sharply where the magnesium content is less than half that of copper and 0.5% each of manganese and nickel are present.

In respect to the effect of varying the proportions of manganese and nickel it is to be seen that although the highest tensile strength is obtained when both elements are present in equal amounts, the difference between such alloys and those containing other proportions is not great.

The effect of exposure of sand cast test bars to a higher temperature, 700° F., is illustrated in the examples given below in Table II. In this case the bars were heated to 700° F., held at that temperature for 48 hours and then tested while at temperature.

TABLE II

Tensile properties of alloy castings at 700° F.

| Composition, Percent |    |     |     | Tensile Strength, p. s. i. | Yield Strength, p. s. i. | Elongation, percent in 2 in. |
|----------------------|----|-----|-----|----------------------------|--------------------------|------------------------------|
| Cu                   | Mg | Mn  | Ni  |                            |                          |                              |
| 8                    | 6  | 0.5 | 0.5 | 10,000                     | 7,000                    | 61                           |
| 14                   | 6  | 0.5 | 0.5 | 15,000                     | 10,000                   | 35                           |

The adverse effect of a higher temperature upon the strength of the alloys is readily apparent, however, it is significant that the tensile and yield strengths of the first alloy tested at 700° F. are only slightly below those of Y alloy at 600° F. Furthermore, a higher copper content is desirable where a temperature of 700° F. is encountered.

The relative constancy of tensile properties at elevated temperatures is often important in service. The effect of long exposure at 600° F. is to be seen in the follow-

ing test where sand cast test bars of an aluminum, 8% copper, 6% magnesium, 0.5% manganese and 0.5% nickel alloy were held at 600° F. for different periods of time and the bars tested at the elevated temperature.

The Brinell hardness values were determined by use of a 10 mm. diameter ball under a 500 kg. load for a period of 30 seconds. The results of the tests are given below in Table III.

TABLE III  
Effect of time on tensile properties at 600° F.

| Time, Hrs. | Tensile Strength, p. s. i. | Yield Strength, p. s. i. | Percent Elongation | BHN |
|------------|----------------------------|--------------------------|--------------------|-----|
| 1/2        | 20,500                     | 16,000                   | 25                 | 43  |
| 10         | 21,500                     | 15,500                   | 25                 | 41  |
| 100        | 19,500                     | 14,500                   | 25                 | 39  |
| 1000       | 19,000                     | 13,500                   | 25                 | 36  |

From the foregoing it will be seen that there was no substantial change in properties between 1/2 and 1000 hours at temperature. This is further evidence of the superiority of our alloy over prior alloys.

The fatigue strength of the foregoing alloy at 600° F. is also important. The fatigue strength values of this alloy at 600° F. as compared with those of Y alloy under the same conditions are given below in Table IV.

TABLE IV

Fatigue strengths at 600° F.

| Number of Cycles | Our Alloy, p. s. i. | Y Alloy, p. s. i. |
|------------------|---------------------|-------------------|
| 10 <sup>4</sup>  | 18,000              | 14,500            |
| 10 <sup>5</sup>  | 14,500              | 11,000            |
| 10 <sup>6</sup>  | 11,000              | 8,500             |
| 10 <sup>7</sup>  | 8,000               | 6,000             |
| 10 <sup>8</sup>  | 6,000               | 4,000             |

Having thus described our invention and certain embodiments thereof, we claim:

1. An aluminum base alloy casting composed essentially of aluminum, 6 to 18% copper, 4 to 8% magnesium, 0.1 to 2% manganese and 0.1 to 2% nickel, the amount of copper not being less than the amount of magnesium, said alloy being characterized in the as-cast condition by a tensile strength at 600° F. of not less than 15,000 p. s. i.

2. An aluminum base alloy casting composed essentially of aluminum, 7 to 11% copper, 5 to 7% magnesium, 0.4 to 1% manganese and 0.4 to 1% nickel, said alloy being characterized in the as-cast condition by a tensile strength at 600° F. of not less than 17,000 p. s. i.

3. An aluminum base alloy casting composed essentially of aluminum, 6 to 16% copper, 4 to 8% magnesium, 0.1 to 2% manganese, 0.1 to 2% nickel, the proportion of magnesium to copper being such that the amount of magnesium is at least one-half the copper content but does not exceed the copper content, said alloy being characterized in the as-cast condition by a tensile strength at 600° F. of not less than 17,000 p. s. i.

4. An aluminum base alloy casting composed essentially of aluminum, 6 to 18% copper, 4 to 8% magnesium, 0.1 to 2% manganese and 0.1 to 2% nickel, the amount of copper not being less than the amount of magnesium, said alloy also containing at least one element selected from the group of grain refining elements consisting of 0.001 to 0.1% boron and 0.01 to 0.2% titanium, said alloy being characterized in the as-cast condition by a tensile strength at 600° F. of not less than 15,000 p. s. i.

5. An aluminum base alloy casting composed essentially of aluminum, 6 to 18% copper, 4 to 8% magnesium, 0.1 to 2% manganese and 0.1 to 2% nickel, the amount of copper not being less than the amount of magnesium, said alloy also containing 0.0001 to 0.1%

beryllium, said alloy being characterized in the as-cast condition by a tensile strength at 600° F. of not less than 15,000 p. s. i.

6. An aluminum base alloy casting composed essentially of aluminum, 6 to 18% copper, 4 to 8% magnesium, 0.1 to 2% manganese and 0.1 to 2% nickel, the amount of copper not being less than the amount of magnesium, said alloy also containing at least one element selected from the group of hardening elements consisting of chromium, cobalt, molybdenum, tungsten, zirconium and vanadium in amounts of 0.1 to 0.6% each

and a total not exceeding 1.0%, said alloy being characterized in the as-cast condition by a tensile strength at 600° F. of not less than 15,000 p. s. i.

References Cited in the file of this patent

UNITED STATES PATENTS

|           |       |       |               |
|-----------|-------|-------|---------------|
| 1,831,584 | Weiss | ----- | Nov. 10, 1931 |
| 1,932,861 | Wood  | ----- | Oct. 31, 1933 |
| 1,940,133 | Kempf | ----- | Dec. 19, 1933 |